

[54] FLUXES FOR USE IN BONDING PLATES OF  
STORAGE BATTERIES TO CONNECTING  
STRAPS

[75] Inventor: Lester Aronberg, Chicago, Ill.

[73] Assignee: Lake Chemical Company, Chicago,  
Ill.

[22] Filed: Mar. 27, 1972

[21] Appl. No.: 238,609

[52] U.S. Cl. .... 148/23, 260/29.6 HN

[51] Int. Cl. .... C23c 1/12

[58] Field of Search..... 148/23, 27; 260/29.6 HN,  
260/29.6 TA, 29.6 WB; 106/181

[56] References Cited

UNITED STATES PATENTS

|           |        |                         |             |
|-----------|--------|-------------------------|-------------|
| 2,898,255 | 8/1959 | Thompson .....          | 148/23      |
| 3,087,005 | 4/1963 | Sabatino et al. ....    | 148/23 X    |
| 3,170,888 | 2/1965 | Kutik et al. ....       | 260/29.6 WB |
| 3,235,414 | 2/1966 | Marks .....             | 148/23      |
| 3,305,406 | 2/1967 | Chmelik et al. ....     | 148/23      |
| 3,424,625 | 1/1969 | Tiegel .....            | 148/23      |
| 3,594,336 | 7/1971 | Bergmeister et al. .... | 260/29.6 TA |

3,736,287 5/1973 Patella..... 260/29.6 TA  
4,314,094 6/1968 JA

FOREIGN PATENTS OR APPLICATIONS

|          |        |                     |        |
|----------|--------|---------------------|--------|
| 481,680  | 3/1952 | Canada .....        | 148/23 |
| 708,921  | 5/1965 | Canada .....        | 148/23 |
| 719,889  | 7/1952 | Great Britain ..... | 148/23 |
| 43-14094 | 6/1968 | Japan .....         | 148/23 |

Primary Examiner—J. Spencer Overholser  
Assistant Examiner—Ronald J. Shore  
Attorney, Agent, or Firm—Wallenstein, Spangenberg,  
Hattis & Strampel

[57] ABSTRACT

Fluxes for use in forming a bond between the lugs of the positive and negative plates, or grids, of a storage battery, and the terminal post-bearing connecting straps thereof, which, in their preferred form, comprise an aqueous suspension of an organic, substantially water-insoluble polycarboxylic acid such as adipic acid, and a water-soluble binder exemplified by polyvinylpyrrolidone.

8 Claims, No Drawings

## FLUXES FOR USE IN BONDING PLATES OF STORAGE BATTERIES TO CONNECTING STRAPS

This invention relates to fluxes for use in forming a bond between the lugs of the positive and negative plates, or grids, of a lead storage battery, and the terminal post-bearing connecting straps of the battery.

In the assembly of the cells of a lead storage battery of the type used in automotive vehicles, it is the practice to bond the lugs of the plates, or grids, which comprise the cells of the battery, to terminal post-bearing connecting straps. The plates, or grids, and the connecting straps are formed of lead alloyed with minor amounts, typically from 3 to 6 percent of antimony, and it is important that the bond formed between the lugs of the plates, or grids, and the connecting straps be strong, otherwise the operation and the useful life of the battery will be adversely affected. Generally speaking, procedures used in attaining a bond require the use of heat to bring about a fusion of the metal of the lugs with the metal of the connecting straps. One such procedure involves preheating the lugs of the plates, or grids, to a temperature of approximately 450°F, and contacting the preheated lugs with the metal of the connecting straps which is held in a mold in a molten condition at a temperature of approximately 925°F. A flux is customarily applied to the lugs prior to contacting them with the molten metal in the connecting strap molds.

Heretofore, fluxes such as zinc chloride and tin chloride, and mixtures thereof, which have been dissolved in water, with or without an acid, such as hydrochloric acid, have been used in forming a bond between the lugs and the molten metal of the connecting straps. These fluxes, however, have been found to be unsatisfactory due, in the main, to their corrosive properties and to their tendency to form oxides, the effect of which is to weaken the bond between the lugs and the connecting straps. These weakened bonds cause heating and resistance in the cells of the battery, and materially shorten the useful life of the battery. In an attempt to overcome the deleterious effects of the corrosive zinc and tin chloride fluxes, it has been proposed to use a solution of an alcohol and rosin as a flux. However, such a flux, while being non-corrosive, is unsatisfactory for a variety of reasons.

In accordance with the present invention, fluxes have been evolved which eliminate the disadvantages of fluxes heretofore used in connection with the bonding of the lugs of plates, or grids, to the connecting straps of storage batteries. Apart from their non-corrosive properties, the fluxes of this invention are characterized by their ability to function at the relatively high temperatures utilized in the bonding operation to provide bonds between the lugs and the connecting straps which are uniformly strong. These objectives are achieved, moreover, without the concomitant production of contaminants or pollutants, airborne or otherwise.

In brief the fluxes of the present invention, in their preferred form, comprise, as essential ingredients, an organic, substantially water-insoluble polycarboxylic acid, and a water-soluble binder. In accordance with an especially preferred practice of the invention, the fluxes are utilized in the form of aqueous dispersions or suspensions, the aqueous phase of the dispersion or suspension acting as a carrier for the particles of the substantially water-insoluble polycarboxylic acid, and as

the solubilizing agent for the binder. The term "polycarboxylic acid" as used herein is intended to encompass acids having 2, or more, preferably 2 to 4, carboxyl groups.

5 The organic polycarboxylic acids useful in the preparation of the fluxes of this invention, apart from being substantially water-insoluble, are characterized in that they will not sublime, or manifest no substantial sublimation, at the temperatures employed in bonding the lugs of battery plates, or grids, to the connecting straps. As indicated hereinabove, these temperatures are of an order of 900°F, more or less. Exemplary of organic polycarboxylic acids which meet the aforementioned desiderata are aliphatic hydrocarbon dicarboxylic acids such as adipic acid and azelaic acid; aromatic dicarboxylic acids specific examples of which are uvitic acid, isouvitic acid, and homophthalic acid; aromatic polycarboxylic acids exemplified by pyromellitic acid; and the like. Of the foregoing acids, adipic acid is outstandingly effective.

20 The binders having utility in the preparation of the fluxes can be selected from various water-soluble gums and resins. Exemplary thereof are water-soluble gums such as gum arabic, cedar gum and cebil gum; water-soluble gun-like compounds exemplified by sodium carboxymethyl celluloses; higher fatty acid partial esters of aliphatic water-soluble polyhydric alcohols or polyhydroxy substances; and water-soluble polymeric materials exemplified by polyvinylpyrrolidone, the latter being particularly preferred as a binder because it serves the added function of improving the wetting, spreading and capillary action of the fluxes.

25 As indicated hereinabove, the fluxes of this invention advantageously are used in the form of aqueous dispersions or suspensions, the water-insoluble organic polycarboxylic acid constituting the dispersed or suspended phase of the dispersion. The distribution of the acid in the dispersion or suspension can be enhanced by reducing, as by grinding, the size of the crystals or particles of the acid. Excellent results can thus be attained with particles having a mesh size of the order of about 40 to about 150, especially desirably about 90 to about 120.

30 45 The quantity of the organic polycarboxylic acid and the binder used in the preparation of the fluxes is somewhat variable. Typically, a flux, in the form of an aqueous dispersion or suspension, will contain from about 10 to 80 percent, usually about 40 to about 60 percent, by weight, of the water-insoluble organic polycarboxylic acid, and from about 0.2 to about 5 percent, especially desirably from about 0.5 to about 2 percent, by weight, of the binder. While tap water can be used to form the dispersions or suspensions, it is desirable to use distilled water for this purpose, especially in those instances where undesirable chemicals may have been introduced into the tap water at a water treatment plant, or by natural processes.

50 55 60 In utilizing the fluxes of the present invention, they are advantageously applied to the lugs of the battery plates, or grids, at ambient temperatures. The flux-coated lugs are then subjected to a preheating operation, after which they are brought into contact with the molten metal of the connecting straps. The fluxes may be applied to the lugs in any convenient manner known to the art as by dipping, spraying, brushing, or the like.

While, as described hereinabove, the fluxes, in their preferred form, contain as essential ingredients, a water-insoluble, organic polycarboxylic acid and a water-soluble binder, in accordance with another, but less preferred, aspect of the present invention, the binder can be eliminated, and the polycarboxylic acid, in a dry, powdered or pulverulent form, can be used alone. When thusly used, the dry, powdered acid advantageously is applied, as by spraying from an aerosol container, or the like, to the surface of the lugs, advantageously after the lugs have been preheated. In accordance with yet another, but also, less preferred aspect of the invention, an inert alcohol or ether can be used in place of water as a carrier for the polycarboxylic acid, with or without the binder. Specific examples of alcohols and ethers which can be used, and which include higher boiling alcohols, are ethanol, isopropanol, hexanol, heptanol, glycerol, and the like, and higher boiling ethers exemplified by methyl cellosolve, ethyl cellosolve, butyl cellosolve, and the like, and compatible mixtures thereof. In utilizing an alcohol or ether as a carrier, suitable steps should be taken to vent any vapors or fumes from the work area.

The following examples are illustrative of the fluxes of this invention. It will be understood that various other fluxes can be made in the light of the guiding principles and teachings disclosed hereinabove. All parts are listed by weight.

EXAMPLE 1:

|                        |      |
|------------------------|------|
| Adipic acid (100 mesh) | 40   |
| Binder (gum arabic)    | 0.5  |
| Water                  | 59.5 |

EXAMPLE 2:

|                                   |      |
|-----------------------------------|------|
| Adipic acid (100 mesh)            | 40   |
| Binder (PVP-polyvinylpyrrolidone) | 0.5  |
| Water                             | 59.5 |

EXAMPLE 3:

|                        |    |
|------------------------|----|
| Azelaic acid (80 mesh) | 60 |
| Binder (PVP)           | 1  |
| Water                  | 39 |

EXAMPLE 4:

|                           |    |
|---------------------------|----|
| Isouvitic acid (100 mesh) | 45 |
| Binder (PVP)              | 2  |
| Water                     | 53 |

EXAMPLE 5:

|                             |    |
|-----------------------------|----|
| Pyromellitic acid (40 mesh) | 70 |
| Binder (PVP)                | 1  |
| Water                       | 29 |

30 5. A water-based flux for use in forming a bond between the lugs of the plates of a lead storage battery and the connecting straps of said plates, consisting essentially of an aqueous suspension of a substantially water-insoluble polycarboxylic acid in particulate form, and a water-soluble binder dissolved in the aqueous phase of the suspension, the polycarboxylic acid being characterized in that it does not undergo any substantial sublimation at the temperatures at which the lugs of the plates of a lead storage battery are bonded to the connecting straps.

35 6. A flux according to claim 1 wherein the aqueous phase of the suspension comprises from about 90 percent to 20 percent, by weight, of the suspension.

40 7. A flux according to claim 1 wherein the binder comprises, by weight, about 0.5 percent to about 2 percent of the suspension.

45 8. A flux according to claim 1 wherein the particles of the acid have a mesh size of from about 40 to about 150.

\* \* \* \* \*